

## UNITED STATES PATENT OFFICE

EUGENE C. GWALTNEY, OF LAUREL HILL, NORTH CAROLINA

## PROCESS FOR THE MANUFACTURE OF COTTON YARN AND IMPROVED PRODUCT

No Drawing.

Application filed July 9, 1927. Serial No. 204,540.

My invention relates to an improved process for the manufacture of cotton yarn, and to an improved product.

The object is to provide increased evenness and uniformity, and breaking strength in the resultant product.

It is well known and accepted that combed yarns are stronger than carded yarns.

In the process of combing, as heretofore practiced, the percentage of waste taken out has been from 10% to 20%. The theory has been that the improvement in breaking strength of combed yarn over carded yarn has been due to the fact that the short fibres were eliminated in the combing process. My experience has shown that improvement in break is due, not so much to the elimination of short fibres but, rather, to a more perfect parallelization of the fibre in the comber. I have proven that a comber using coarser needles with a wider spacing between the needles taking out a larger percentage of waste will not give a breaking strength in any way equal to that produced on a comber in which the needles are fine and closely set taking out a waste percentage of not over 2%, thus demonstrating that the increase in break is due rather to the perfect straightening of the fibre than to the elimination of short fibre.

In my process, the combed sliver used is produced with the smallest possible amount of fibres removed and for the purposes of straightening and parallelizing the fibres and improved cleanliness.

In my improved process and product, I combine both combed and carded fibres into slivers, and in that way overcome the unevenness due to the piecings inherent in the combed sliver process referred to and get a more uniform distribution of the fibres, thus taking advantage of, and utilizing, the more uniform distribution of the fibres well known to exist in the ordinary carded sliver, and also the more perfect parallelized fibres in combed sliver which assists in the subsequent drafting of the carded sliver in the manufacture of the finished yarn.

The blending of the more uniform and evenly carded sliver with the combed sliver tends to eliminate the unevenness and to dis-

tribute the fibres more uniformly throughout the cross-section of the resultant yarn or thread.

It has been found that by the blending of carded and combed sliver in the manufacture of cotton yarn that the breaking strength of the resulting yarn has been materially increased over the breaking strength of either the combed or the carded yarn alone. In other words, the blending of the two gives a stronger yarn than either of the two are when spun separately. For instance on carded one and three-sixteenth inch cotton spun and twisted in a tire fabric cord, the breaking strength of the carded yarn or cord is seventeen and one-half pounds; of the combed, it was eighteen; for the blended, that is the combed and carded, eighteen and one-half pounds. These tests were all made by a member of the American Society for Testing Materials, who is also a member of the Tire Fabric Committee, with the latest approved testing-machines corrected for moisture regain, the tests all having been made in the laboratory where the atmospheric conditions were maintained to give the standard regain of six and one-half per cent, all in accordance with the regulations, as laid down by the above-named society for testing cord fabric. Tests of the single yarns give practically the same result.

In the foregoing process, as now operating, the percentage of waste on the combed fibres is held down from ten per cent to less than two per cent, which latter waste percentage makes a yarn cost but very little more than a carded yarn, while in strength it is much superior to a combed yarn.

Also I get the following improvement on carded yarns: Increasing cleanliness and greater lustre due to the combing operation, better drafting qualities in subsequent process as compared with carded sliver due to superior parallelization of fibres making possible very much longer drafts than can be used with carded sliver with no decrease in breaking strength with the resulting economy in manufacture due to increased drafts.

I claim:

1. An improved process in which the card-

100

ed and combed cotton slivers or rovings are combined in the formation of a thread, yarn, twine or card, to give an increased strength to resulting product.

2. An improved process in which the carded and combed cotton slivers or rovings are combined in the formation of a thread, yarn, twine or cord in which the waste from the combed sliver does not exceed ten per cent, to give an increased strength to resulting product.

3. A thread, yarn, twine or cord composed of a blending of combed and carded cotton fibers to give an increased strength to resulting product.

4. A thread, yarn, twine or cord composed of a blending of combed and carded cotton slivers, in which the waste from the combed sliver is held so low as to not materially increase the cost of resulting product though resulting in greater strength.

5. As a new process, the blending together of carded and combed cotton slivers or fibers.

6. As a new process of manufacture, the blending together of carded and combed cotton slivers or fibers in the formation of a thread, yarn, twine or cord.

In testimony whereof I affix my signature.  
EUGENE C. GWALTNEY.

30

35

40

45

50

55

60

65